

## UNITED STATES PATENT OFFICE

2,004,472

## PRODUCTION OF LEATHER

George R. Pensel, Amsterdam, N. Y.

No Drawing. Application May 29, 1931,  
Serial No. 541,122

4 Claims. (Cl. 149—3)

This invention relates to processes of preparing leather.

More specifically, it is directed to a novel treatment of skins preliminary to the actual tanning operation, which contributes to the production of leather of excellent quality.

As far as I am aware, no one up to the present time has been commercially successful in producing tough, pliable leather having the grain left thereon by any process employing formaldehyde. The leather resulting from previous attempts has been hard and brittle. Accordingly, an object of the present invention is to provide a tannery process using formaldehyde which will produce grain leather acceptable to the trade. It is to be understood, however, that the instant process is excellently suitable for the production of leather from all classes of skins, including lizard and snake skins, shearlings and furs.

Other and further objects of the present invention will be apparent to those skilled in the art upon studying the present specification and claims.

According to methods now in use, skins as received at the tannery pickled in sulfuric acid and salt, are treated with sodium bicarbonate, borax, whiting, etc., to neutralize the strong acid prior to the actual tanning operation. According to the present invention and constituting an important feature thereof, the strong acid is not neutralized directly but is converted into or replaced by a weak organic acid which is then neutralized to a pH number of about 5.2 to 6.0 by the addition of an agent such as sodium bicarbonate or borax. The strong acid is removed by treating the skins with a soluble salt of a weak organic acid, such as an alkali metal salt of acetic, oxalic, lactic, tartaric, citric, formic and other such weak acids, which salt reacts with the strong acid to form the weak organic acid and inorganic salt. It is desirable in the treatment of most skins to add to the treatment bath a quantity of the organic acid itself.

After the neutralization step the skins are in condition for the tanning or tawing operation. The preliminary treatment explained above beneficially affects the leather produced no matter what the actual tanning operation may be. However, the preliminary treatment is particularly of value to the leather produced when the tanning or tawing is effected by the use of an aldehyde. And further, the best results are obtained when the formaldehyde tannage is of the particular nature hereinafter described in detail.

This particular tanning operation is performed

by subjecting the neutralized skins to a treatment at a slightly elevated temperature with a bath composed of a solution of formaldehyde, Glauber's salt, borax and a substance which assists the formaldehyde in entering the skins, such as a sodium soap or a small amount of emulsified olive, cocoanut, or sperm oil, or mixtures of sulphonated oils, preferably castor, cocoanut and sperm. The skins are then washed, and bleached, if necessary.

The novel fat liquoring treatment which follows, though quite important to the successful production of some leathers such as grain leather, is not of so much importance to others. When grain leather is treated, it is heated at a slightly elevated temperature in a bath containing a sulphonated mixture of sperm and cocoanut oils. When suedes are treated, sulphonated castor oil is added to the bath. After a treatment with weak acetic acid and a washing operation, the skins are ready for finishing.

Other aldehydes than formaldehyde may be successfully employed, for instance, acrolein.

As an example of the complete process of the present invention, a typical run in which doeskins are tanned is herein set out, the quantities of substances used being those amounts employed per one hundred pounds of pickled skins.

The pickled skins as received, which contain sulphuric acid, are fleshed and degreased, as, for example, with kerosene, and then soaked and agitated in a drum having therein a water solution containing about 5 to 6 pounds of sodium acetate and about 20 to 24 pounds of Glauber's salt for each twenty gallons of water. The agitation is continued for a period of about a half hour at a temperature in the neighborhood of 80° F.

In some cases where the skins contain an unusual or excess amount of sulphuric acid, a somewhat larger amount of sodium acetate should be used. Also for grain leather skins the amount of Glauber's salt above indicated should be substantially increased even up to fifty pounds.

To the drum may then be added 2 to 6 pounds of 56% acetic acid in a solution containing a small additional quantity of Glauber's salt, after which the soaking and agitating is continued for about another half hour. The solution now has a pH value of approximately 5.2.

Next, the acetic acid solution is neutralized by adding about 2 to 3 pounds of bicarbonate of soda, or the equivalent in borax, in solution in water containing additional Glauber's salt. This raises the pH number of the solution to approxi-

mately 5.5. After a run of about a half hour, with the temperature still about 80° F., the skins are slatted off and the liquid drained away.

Then the actual tanning operation begins. A solution containing about 6 to 7 pounds of formaldehyde (40% solution) and 3 to 5 pounds of borax is then added to the drum and run for about an hour at about 80° F. Additional acetic acid is then added to the tanning solution. This lowers the pH value by producing boric acid. To the solution is then added an agent which produces a colloidal condition in the tanning solution which in turn aids the penetration of the formaldehyde. In the present case, this agent is a sodium soap containing, for example, 88% neutral soap made from cocoanut oil and white tallow in about equal proportions, and about 10% of Glauber's salt. The contents are then heated to a boiling temperature and cooled to about 120° F. in about an hour, after which a heating at temperatures gradually increasing to 140° F. over a period of about two hours is effected. This heating may be carried out by running for an hour during a temperature increase from 120 to 130° F., running at 130° F. for a half hour, and at temperatures increasing to 140° F. for an additional half hour, at which time the tanning is complete. The skins are next washed and then bleached if necessary.

The following fat liquorizing process has been found excellently suitable for the production of soft and pliable leather from the skins tanned by the foregoing process. In the treatment of grain leather, the tanned skins are heated at about 125° F. for a half hour in a drum containing about 10 pounds of a sulphonated mix-

ture of equal parts of sperm and cocoanut oils dispersed in water. About 5 pounds of 28% acetic acid dissolved in water is then added gradually to the drum over a period of about a half hour. The treated leather is next washed for about 20 minutes at a temperature of about 100 F., after which the leather is ready for finishing.

Having thus described the invention, what is claimed as new and desired to be secured by Letters Patent is:

1. In the production of leather from skins pickled in strong acid of the pickle solution, the step comprising replacing the strong acid in said skins with acetic acid, and then converting the skins into leather by a formaldehyde tannage process.

2. In the production of leather from skins pickled in strong acid, the steps comprising soaking said skins in a solution containing an alkali salt of acetic acid, neutralizing the acid in the skins to approximately pH 5, and converting the skins into leather by treatment in a bath containing formaldehyde and borax.

3. In the production of leather from skins pickled in strong acid, the steps comprising replacing the strong acid of the pickled solution in the skins with a soluble fatty organic acid, and then converting the skins into leather by the formaldehyde tannage process.

4. In the process of producing leather from skins, the steps of treating the skins with a salt of an organic acid together with a quantity of said organic acid, and then converting the skins into leather by a formaldehyde tannage process.

GEORGE R. PENSEL.